

## UNITED STATES PATENT OFFICE

JOHN A. GANN AND JAMES B. REID, OF MIDLAND, MICHIGAN, ASSIGNORS TO THE DOW CHEMICAL COMPANY, OF MIDLAND, MICHIGAN, A CORPORATION OF MICHIGAN

## METHOD OF CASTING MAGNESIUM AND ALLOYS THEREOF

No Drawing.

Application filed May 4, 1932. Serial No. 609,281.

The present invention relates to methods of casting readily oxidizable metals, particularly magnesium and alloys thereof wherein the magnesium content predominates. One object of the present invention is to permit casting such metals in moist or "green" sand molds and the like, whereby the metal is protected from attack by air or by the steam generated in the mold when the hot metal is poured. Another object of our invention is to produce castings of the aforementioned metals the surface of which has a good appearance and is substantially free from burned spots, pits, or other defects which result from casting such metals in ordinary water-bound molds. Other objects and advantages will appear as the description proceeds.

For convenience, the term "magnesium" is used herein and in the appended claims to mean not only pure magnesium but also alloys of the same in which the magnesium content predominates.

Magnesium, as is well known, has a high affinity for oxygen which is very pronounced when the metal is hot. The casting of this metal in sand molds of the ordinary type used in casting other metals, such as iron, aluminum, copper, is unsatisfactory since the oxygen in the mold acts to oxidize or burn the hot metal, and where the mold is water-bound, as in conventional practice, the metal will decompose the water and combine with the oxygen thereof to such an extent that, if the casting is of relatively heavy section, it may be largely or completely burned up. Many attempts have been made to discover ways of overcoming this difficulty, particularly in an effort to find suitable agents that could be added to molding compositions, such as water-bound or "green" sand, which would overcome this inherent tendency of magnesium and its alloys to oxidize and burn when cast. However, in spite of the extensive work done in this field, only a very few agents have been found that can be so used with any degree of success. For instance, United States Patent No. 1,825,242 discloses the use of ammonium fluosilicate as an agent to prevent

burning of magnesium in a water-bound sand mold and, at the same time by the chemical action of the protective substance, to produce on the surface of the casting a film of a fluorine compound to increase the 55 resistance to corrosion of the casting. Our experimental work in connection with the aforementioned ammonium fluosilicate, however, has shown that its use as a protective agent is not wholly satisfactory. For instance, we have found that the effective life of this agent in the sand is comparatively limited owing to its volatile nature and its tendency to decompose, thereby liberating 60 ammonia, especially when the sand is heated 65 during the casting process. This necessitates frequent re-addition of the agent to the molding sand mixture in order to maintain its effectiveness to prevent burning of the metal. Moreover, accurate mold impressions in molding sand containing this agent may not easily be retained owing to the sand mixture swelling due to chemical reaction 70 between the agent and the wet sand.

As a result of further investigation, we 75 have now made the discovery that a more satisfactory water-bound sand mold for casting magnesium can be produced from molding sand which has been treated with a relatively small amount of a fluosilicate of one 80 of the metals magnesium, lead, sodium, or aluminum. These salts are relatively stable and are not vaporized out of the molding material at the temperatures existing in the sand molds in which magnesium is cast. Accordingly, the foundry sand which has been treated with a metallic fluosilicate may be used repeatedly without becoming materially impoverished with respect to the protective 85 agent. Numerous tests with water-bound molds made from foundry sand treated with a metallic fluosilicate of the character in hand definitely show that castings which cannot ordinarily be made without imperfections 90 where other agents, such as ammonium salts, sulphur, or boric acid, are used, can be satisfactorily cast where our aforementioned metallic fluosilicates are used, as hereinafter set forth.

Accordingly, the present invention pro- 100

vides a procedure for casting readily oxidizable metals, such as magnesium, in water-bound temporary molds, whereby burning of the metal is prevented. The invention 5 likewise includes an improved water-bound mold for use in casting such metals. To the accomplishment of the foregoing and related ends, the invention, then, consists of the method and improved molds hereinafter 10 fully described and particularly pointed out in the claims, the following description setting forth in detail several forms of molds and modes illustrating, however, but several 15 of the various ways in which the principle of the invention may be used.

While the present invention is applicable for use in connection with various molding materials (sand, carbon, graphite, etc.) for metal casting in general, we will, for simplicity, describe the invention in terms of using 20 our improved oxidation inhibitor agents in water-bound "green" (plastic) sand molding compositions.

The principle of our invention comprises 25 providing, at least in surface exposure in the mold, one of the metallic fluosilicates, viz., aluminum fluosilicate,  $Al_2(SiF_6)_3$ ; lead fluosilicate,  $PbSiF_6 \cdot 2H_2O$ ; magnesium fluosilicate,  $MgSiF_6 \cdot 6H_2O$ ; sodium fluosilicate, 30  $Na_2SiF_6$ . A preferable mode of carrying out our invention consists in forming an intimate mixture of the molding material and a relatively small amount of a compound above-mentioned, tempering the mixture with 35 water, forming said mixture into a mold, and then casting magnesium therein. In addition to said mode of procedure, we may further apply to the inner surfaces of the mold said agents in powder form or in the form of an 40 aqueous solution or emulsion of the same.

The amount of such metallic fluosilicates to mix with the molding composition depends to some extent upon the nature of the casting to be made and the quality of the molding 45 material. In making large castings it is preferable to employ a greater proportion of the inhibitor than when relatively small castings are made. However, since our new agents are comparatively stable and do not 50 decompose to any material extent when heated in the mold, satisfactory small castings may be made in the sand prepared for making large castings, thus obviating the need for having different batches of molding 55 sand mixtures for each class of casting. The actual quantity of one or more of the agents, viz., aluminum fluosilicate, lead fluosilicate, magnesium fluosilicate, sodium fluosilicate, to incorporate in the molding material may 60 vary from to 1 to 10 per cent by weight of the sand or other suitable molding material according to the size of the casting. Under ordinary conditions, an amount of the agent greater than the minimum stated should be 65 used unless the casting be made of relatively

thin section throughout. The maximum stated, on the other hand, is adapted for use mainly in the production of castings of exceptionally heavy section throughout. The preferable amount to use is from 2 to 6 per cent, and the addition of approximately 4 per cent, which is well adapted to meet ordinary casting needs, enables sound clean castings to be made in water-bound sand molds. When employing such agents as a mixture of 70 more than one of the same, the total quantity of such mixture added to the molding material may be preferably within limits specified above.

Naturally the effectiveness of any oxidation inhibitor for use as hereinbefore described varies with the permeability of the sand, being somewhat greater with sands of high permeability than with those of relatively low permeability. The molding sand should, therefore, be sufficiently open or permeable to permit of free escape of gases out of the mold, which are formed by contact with the hot metal as it is poured into the mold. In general we have found that a permeability factor of 30 or more gives satisfactory results, although in many cases good results may be obtained with sands of somewhat lower permeability. The definition of the term "permeability" as used herein and the method of measuring its numerical value is described in the bulletin "Testing and Grading Foundry Sands", published by the American Foundrymen's Association, March 1931.

The protective effect of our new agents is materially greater than that of ammonium fluosilicate. For example, a magnesium casting weighing 9 pounds was cast in a water-bound sand mold to which was added 3 per cent of ammonium fluosilicate. Result: 100 casting showed surface defects in the form of burned spots, indicating inadequate protection from oxidation by the water in the mold. The same magnesium casting was cast in a similar manner and in similar foundry sand except that 3 per cent of magnesium fluosilicate was employed as oxidation inhibitor instead of ammonium fluosilicate. The result 105 was a clean, perfect casting. Similar results were obtained by the use of the fluosilicates of aluminum, lead, or sodium, and mixtures thereof.

In the method of casting herein described, it is to be understood that the choice of oxidation inhibitor need not be limited alone 110 to those disclosed, inasmuch as other sand addition agents which are known to give a substantial amount of protection against oxidation of magnesium may be used in conjunction with the improved agents hereinbefore described.

Other modes of applying the principle of our invention may be employed instead of those explained, change being made as regards the means and steps herein disclosed,

provided those stated by any of the following claims or their equivalent be employed.

We therefore particularly point out and distinctly claim as our invention:—

5. 1. The method of making a casting of magnesium or an alloy thereof which comprises casting the metal in a water-bound temporary mold having on the surface thereof a relatively small amount of a compound selected from the group consisting of aluminum fluosilicate, lead fluosilicate, magnesium fluosilicate, sodium fluosilicate. 70
10. 2. The method of making a casting of magnesium or an alloy thereof which comprises forming an intimate mixture of foundry sand and a relatively small amount of a compound selected from the group consisting of aluminum fluosilicate, lead fluosilicate, magnesium fluosilicate, sodium fluosilicate, forming said mixture into a mold, and casting magnesium therein. 75
15. 3. The method of making a casting of magnesium or an alloy thereof which comprises forming an intimate mixture of foundry sand tempered with water and a relatively small amount of a compound selected from the group consisting of aluminum fluosilicate, lead fluosilicate, magnesium fluosilicate, sodium fluosilicate, forming said mixture into a mold, and casting magnesium therein. 80
20. 4. The method of making a casting of magnesium or an alloy thereof which comprises forming an intimate mixture of foundry sand tempered with water and a compound selected from the group consisting of aluminum fluosilicate, lead fluosilicate, magnesium fluosilicate, sodium fluosilicate, forming said mixture into a mold, and casting magnesium therein. 85
25. 5. The method of making a casting of magnesium or an alloy thereof which comprises forming an intimate mixture of foundry sand tempered with water and a compound selected from the group consisting of aluminum fluosilicate, lead fluosilicate, magnesium fluosilicate, sodium fluosilicate, forming said mixture into a mold, applying a compound named in the said group to the inner surface of the mold, and casting magnesium therein. 90
30. 6. The method of making a casting of magnesium or an alloy thereof which comprises forming an intimate mixture of foundry sand tempered with water and from 1 to 10 per cent of a compound selected from the group consisting of aluminum fluosilicate, lead fluosilicate, magnesium fluosilicate, sodium fluosilicate, forming said mixture into a mold, and casting magnesium therein. 95
35. 7. The method of making a casting of magnesium or an alloy thereof which comprises forming an intimate mixture of foundry sand tempered with water and from 2 to 6 per cent of a compound selected from the group consisting of aluminum fluosilicate, lead fluosilicate, magnesium fluosilicate, sodium fluosilicate, forming said mixture into a mold, and casting magnesium therein. 100
40. 8. The method of making a casting of magnesium or an alloy thereof which comprises forming an intimate mixture of foundry sand tempered with water and from 2 to 6 per cent of a compound selected from the group consisting of aluminum fluosilicate, lead fluosilicate, magnesium fluosilicate, sodium fluosilicate, forming said mixture into a mold, and casting magnesium therein. 105
45. 9. The method of making a casting of magnesium or an alloy thereof which comprises forming an intimate mixture of foundry sand tempered with water and from 2 to 6 per cent of a compound selected from the group consisting of aluminum fluosilicate, lead fluosilicate, magnesium fluosilicate, sodium fluosilicate, forming said mixture into a mold, and casting magnesium therein. 110
50. 10. The method of making a casting of magnesium or an alloy thereof which comprises forming an intimate mixture of foundry sand tempered with water and from 2 to 6 per cent of a compound selected from the group consisting of aluminum fluosilicate, lead fluosilicate, magnesium fluosilicate, sodium fluosilicate, forming said mixture into a mold, and casting magnesium therein. 115
55. 11. In a method of casting magnesium or an alloy thereof the steps which consist in applying to the surface of a water-bound temporary mold a facing comprising a compound selected from the group consisting of aluminum fluosilicate, lead fluosilicate, magnesium fluosilicate, sodium fluosilicate, and casting magnesium in said mold. 120
60. 12. A mold for casting magnesium or an alloy thereof formed from the mixture which comprises foundry sand tempered with water and intimately mixed with a compound selected from the group consisting of aluminum fluosilicate, lead fluosilicate, magnesium fluosilicate, sodium fluosilicate. 125
65. 13. A mold for casting magnesium or an alloy thereof formed from the mixture which comprises foundry sand tempered with water and intimately mixed with from 2 to 6 per cent of a compound selected from the group consisting of aluminum fluosilicate, lead fluosilicate, magnesium fluosilicate, sodium fluosilicate. 130

silicate, lead fluosilicate, magnesium fluosilicate, sodium fluosilicate, forming said mixture into a mold, and casting magnesium therein.

8. The method of making a casting of magnesium or an alloy thereof which comprises forming an intimate mixture of foundry sand tempered with water and from 2 to 6 per cent of aluminum fluosilicate, forming said mixture into a mold, and casting magnesium therein. 75

9. The method of making a casting of magnesium or an alloy thereof which comprises forming an intimate mixture of foundry sand tempered with water and from 2 to 6 per cent of lead fluosilicate, forming said mixture into a mold, and casting magnesium therein. 80

10. The method of making a casting of magnesium or an alloy thereof which comprises forming an intimate mixture of foundry sand tempered with water and from 2 to 6 per cent of magnesium fluosilicate, forming said mixture into a mold, and casting magnesium therein. 85

11. In a method of casting magnesium or an alloy thereof the steps which consist in applying to the surface of a water-bound temporary mold a facing comprising a compound selected from the group consisting of aluminum fluosilicate, lead fluosilicate, magnesium fluosilicate, sodium fluosilicate, and casting magnesium in said mold. 90

12. A mold for casting magnesium or an alloy thereof formed from the mixture which comprises foundry sand tempered with water and intimately mixed with a compound selected from the group consisting of aluminum fluosilicate, lead fluosilicate, magnesium fluosilicate, sodium fluosilicate. 100

13. A mold for casting magnesium or an alloy thereof formed from the mixture which comprises foundry sand tempered with water and intimately mixed with from 2 to 6 per cent of a compound selected from the group consisting of aluminum fluosilicate, lead fluosilicate, magnesium fluosilicate, sodium fluosilicate. 110

Signed by us this 29th day of April, 1932.

JOHN A. GANN.  
JAMES B. REID.